

W. M. FRASER.  
PROCESS FOR THE MANUFACTURE OF BITUMINOUS EMULSIONS.  
APPLICATION FILED OCT. 24, 1917.

1,258,103.

Patented Mar. 5, 1918.



**FIG. II.**



Witnesses

Witnesses  
John G. Berger  
James H. Bell.

William M. Fraser,  
by *Feeley & Page* -  
Attorney

# UNITED STATES PATENT OFFICE.

WILLIAM M. FRASER, OF WOODBRIDGE, NEW JERSEY, ASSIGNOR TO THE BARBER ASPHALT PAVING COMPANY, OF PHILADELPHIA, PENNSYLVANIA, A CORPORATION OF WEST VIRGINIA.

## PROCESS FOR THE MANUFACTURE OF BITUMINOUS EMULSIONS.

1,258,103.

Specification of Letters Patent.

Patented Mar. 5, 1918.

Application filed October 24, 1917. Serial No. 198,299.

To all whom it may concern:

Be it known that I, WILLIAM M. FRASER, a citizen of the United States, and a resident of Woodbridge, in the county of Middlesex and State of New Jersey, have invented certain new and useful Improvements in Processes for the Manufacture of Bituminous Emulsions, whereof the following is a specification, reference being had

10 to the accompanying drawings.

My invention relates to bituminous emulsions such as are used in the paving and roofing arts. They are useful because the emulsion being miscible with water in all proportions, may be brought to any required degree of fluidity. Their composition must be such that after a time, they become, as the result of evaporation, immiscible in water, and, therefore, useful as

20 a waterproof binder or cement.

In order to secure a bituminous emulsion useful for these purposes having these qualities, it is necessary to obtain a very thorough emulsification, and on a comparatively large scale. My invention relates to a process for accomplishing this, which is both economical and practical, and it has for its characteristic the simultaneous pumping and mixing of the bituminous substance

30 and the soapy substance, whereby the two are mixed in proper proportions, and their continued pumping after being thus mixed until the required emulsion is secured.

In the practice of my process I find it convenient to employ an apparatus, such as I have shown in the accompanying drawings, in which Figure I, is a plan view and Fig. II, an elevation of such apparatus.

In this apparatus three containers are mounted in close proximity to each other. These are a bitumen tank 1, a soap tank 2, and a mixing tank 3. By suitable valved pipe connections 4, 4, 4, 4, all of these tanks are connected with the suction end of a pump 5. The delivery end of this pump discharges through a pipe 6, into the top of the mixing tank. There is also provided a pipe 7, for a water supply to the mixing tank.

I will now describe a typical process of

50 making a bituminous emulsion in accordance

with my invention, it being understood that the materials and proportions may be varied, and that the data are given by way of example, rather than by way of limitation.

In order to conveniently and cheaply prepare a bituminous emulsion, consisting of a mixture of semi-liquid bitumens or of oils, and watery solutions of soap which will not separate between the freezing and boiling point of water in less than thirty days, 55 and which are miscible in all proportions with water, I take, for instance, Mexican residuum, after the naphthas and burning oils, etc., have been removed, and warm it in tank 1, to a temperature of 180 to 190° F. 60 I take caustic soda, 2.3 parts and fresh water 5.7 parts, and prepare a soda solution having a gravity of 35° Baumé. To this soda solution I then add in small increments 4.5 gallons of rosin oil per each .75 gallon soda 65 solution and stir the batch actively until a smooth solution of soap is produced. To this soap solution I then add 5.5 gallons of additional water and the final and finished soap solution, then has a gravity of approximately 1.1° Baumé. This is placed in tank 2. 70

Having thus provided a supply of asphaltic residuum and of soap solution in tanks 1, and 2, respectively, I pass these simultaneously through the pump 5, preferably in the proportion of 75.5 gallons residuum to 11 gallons soap solution. This mixing operation is begun by opening the cock of the container 1, as well as the cock of the container 80 2, to such a degree that when the pump is started, it will draw both residuum and soap solution simultaneously and in the desired proportions, and pass them through the pump and discharge them into the mixing 85 tank 3. After the initial mixture has been thus made, the connections of the pump with the tanks 1, and 2, are closed, and in place thereof the connection between the base of the mixing tank and the pump is opened, 90 thus permitting the pump to continue the mixing operation by drawing the mixed solution from the bottom of the mixing tank 95 and again discharging it into the top. While this circulation of the mixture is taking 100

place, an additional quantity of water, say 30 or 35 gallons, is gradually added directly to the mixture by means of the pipe 7.

- An alternative method of procedure which 5 I have also found very successful is the following: Having prepared the bituminous material and the soap solution in their respective tanks, in quantities representing the ultimate proportions of the mixture which 0 is desired, I first pump the entire soap solution into the empty mixing tank. Suction is thereupon taken from the bottom of the mixing tank and simultaneously from the tank 1, containing the asphaltic residuum. 5 The mixed material is delivered by the pump into the mixing tank at the top, the bituminous material being thus gradually added to the circulating soap solution. This proceeds until the entire quantity of residuum 0 has been mixed with the soap solution. There may be added from time to time an amount of water on top of the mixture in the mixing tank, a procedure sometimes necessary when the hot mixture causes evaporation which reduces the amount of water 5 which is necessary to get the required results.

In either case the pumping, and, therefore, the mixing operation is continued un-

til the emulsion when tested with a drop of 30 water turns to a light brown color at the point of contact.

Having thus described my invention, I claim:

1. The process of making a bituminous 35 emulsion, which consists in simultaneously pumping from their respective containers a liquid bitumen and an emulsifier, passing them simultaneously through the pump and back to a mixing tank, drawing the mixture 40 off again from the mixing tank to the pump and back again until the entire solution has reached the proper stage of emulsification as a result of continuous pumping.

2. The process of making a bituminous 45 emulsion, which consists in pumping a soapy solution from its tank and simultaneously pumping a liquid bitumen so that the two unite before passing through the pump.

In testimony whereof I have hereunto 50 signed my name, at Philadelphia, Pennsylvania, this twenty-second day of October, 1917.

WILLIAM M. FRASER.

Witnesses:

JAMES H. BELL,  
E. L. FULLERTON.